

# UNITED STATES PATENT OFFICE.

HIRAM STEVENS MAXIM, OF LONDON, ENGLAND.

## MANUFACTURE OF GUNS.

SPECIFICATION forming part of Letters Patent No. 376,990, dated January 24, 1888.

Application filed October 4, 1887. Serial No. 251,389. (No model.) Patented in England March 22, 1887, No. 4,320.

*To all whom it may concern:*

Be it known that I, HIRAM STEVENS MAXIM, mechanical engineer, a citizen of the United States of America, and a resident of London, England, have invented new and useful Improvements in the Manufacture of Guns, (for which I have obtained a patent in Great Britain, No. 4,320, bearing date March 22, 1887,) of which the following is a specification.

10 My invention relates to the manufacture of steel guns, and is designed to provide for increasing the strength of the same and the homogeneity of the metal of which they are composed.

15 Steel guns have in some instances been manufactured from solid castings or ingots by forging the same to the required external shape and roughly boring them, then tempering or toughening the same by heating them in a furnace, and when heated to the required temperature plunging them in oil, and then finishing them. In the manufacture of a gun in this manner the requisite number of "units of work" are put into the steel by hammering 20 or drawing, which is disadvantageous, for the reasons hereinafter explained. Moreover, the metal is liable to warp and crack in the process of tempering or toughening the same. By the term "units of work" I mean the amount 25 of hammering or other working to which the steel must be subjected in order to impart the desired toughness and density thereto. For instance, if the ingot is hammered or drawn until it has been increased to twice its original 30 length, one unit of work is said to have been put into the metal. If the ingot is hammered or drawn until it has been increased to four times its length, three units of work are said to have 35 put into the metal.

40 An important object of my present invention is to provide for putting any desired number of units of work into the metal of which the gun is composed without the necessity for hammering or drawing or changing the form of the 45 ingot for this purpose. I accomplish this result by twisting the steel casting or ingot while hot and before the same is forged, bored, or otherwise worked. In this manner, moreover, I insure that the grain or fiber of the 50 metal shall extend in the direction calculated to give the greatest strength to the gun—that

is to say, that the grain or fiber shall extend circumferentially or spirally around the bore. I can thus produce guns of very great strength as compared with those in which the requisite 55 number of units of work are put into the steel by hammering or drawing. Moreover, the twisting of the casting or ingot insures uniformity in the distribution of the carbon and increases the homogeneity of the metal. 60

Another object of my said invention is to provide for imparting to the gun a molecular condition, such as that which exists in a built-up gun—that is to say, for insuring that the inner portions of the gun shall be under compression while the outer portions thereof are 65 in a state of tension. For this purpose I first temper or toughen the gun in the ordinary manner, and then reheat the same, and while it is still in the furnace I cool it from the interior by means of air, water, oil, or other suitable cooling medium. 70

In making a gun according to my present invention I proceed as follows—that is to say: I take a steel casting or ingot of the requisite 75 dimensions, and twist the same while hot by means of a lathe or other suitable machine until the desired number of units of work has been put into the steel. This twisting is preferably so effected that it does not lengthen the 80 ingot. The ingot may then be bored to the required caliber, turned, and otherwise finished; or it may be hammered or drawn to lengthen it before being bored. 85

I find it advantageous to subject the casting 90 or ingot thus twisted to the further operations herein after described—that is to say, I forge the said ingot to the required external shape or configuration, and then roughly bore the same and temper or toughen it by means of oil in the ordinary manner, the cooling being effected from the outside as well as from the inside of the gun. I then heat the gun to a red heat, and while it is still in the furnace and its exterior is subjected to heat I cool it 95 internally, using for this purpose a blast or current of cold air, or of air and steam, or of air having in suspension therein water in a finely-divided or atomized condition, or a blast or current of air combined with a spray of oil, 100 or a stream of oil or of hot or cold water, the means employed being varied according to the

nature or the desired hardness of the steel, the dimensions of the gun, and other circumstances. I then finish the gun in any convenient manner.

In some instances I repeat as often as may be required the operations of tempering or toughening the gun in the ordinary manner and of cooling the gun internally while subjected to heat externally, as above described, for the purpose of improving the quality of the steel.

It is evident that by twisting the ingot, instead of hammering or drawing the same, to put the desired number of units of work into the metal, the effect of any air-hole or other fault in the metal will be diminished instead of increased. For instance, assuming a fault—such as a spot containing too much or too little carbon—to exist in the ingot, the hammering or drawing would lengthen the said fault or draw it out lengthwise of the gun, thereby diminishing the resistance of the gun to internal pressure, whereas by the twisting of the ingot the fault is drawn out circumferentially, so that the strength of the gun to resist internal pressure will be increased.

I can, if desired, take a hollow casting and twist it, in the manner above described, until any desired number of units of work is put into the steel, the said hollow casting being subsequently forged, if necessary, tempered or toughened, and finished, as above specified.

What I claim is—

1. The improvement in the manufacture of steel guns, which consists in twisting the steel casting or ingot to be used in making the gun, as and for the purpose set forth.

2. The improvement in the manufacture of steel guns, which consists in twisting the steel casting or ingot to be used in making the gun and then cooling it internally, as set forth.

3. The improvement in the process of mak-

ing steel guns, which consists in twisting the steel casting or ingot to be used in making the gun and then heating and cooling it internally.

4. The improvement in the process of making steel guns, which consists in twisting the steel casting or ingot to be used in making the gun, boring the casting or ingot when cast solid, and then cooling it internally while its exterior is exposed to heat.

5. The improvement in the process of making steel guns, which consists in twisting the steel casting or ingot to be used in making the gun, boring the same when cast solid, then tempering or toughening it in the ordinary manner, and then reheating it and cooling it internally while its exterior is exposed to heat, as set forth.

6. The improvement in the process of making steel guns, which consists in twisting the steel casting or ingot to be used in making the gun, then forging the said casting or ingot to the desired shape or configuration, then roughly boring the same, and then heating it and cooling it internally while its exterior is exposed to heat, as set forth.

7. The improvement in the process of making steel guns, which consists in twisting the steel casting or ingot to be used in making the gun, then forging the said casting or ingot to the desired shape or configuration and roughly boring the same, then tempering or toughening it in the ordinary manner, and then reheating it and cooling it internally while its exterior is exposed to heat.

In testimony whereof I have hereunto signed my name in the presence of two subscribing witnesses.

HIRAM STEVENS MAXIM.

Witnesses:

DAVID YOUNG,  
WALTER MORRIS.